

# UNITED STATES PATENT OFFICE.

CARL SPÄTH, OF STEGLITZ, NEAR BERLIN, GERMANY, ASSIGNOR TO EASTMAN KODAK COMPANY, OF ROCHESTER, NEW YORK, A CORPORATION OF NEW YORK.

## PROCESS FOR THE MANUFACTURE OF COLOR-SCREENS.

1,081,341.

Specification of Letters Patent. Patented Dec. 16, 1913.

No Drawing.

Application filed October 14, 1910. Serial No. 587,062.

To all whom it may concern:

Be it known that I, CARL SPÄTH, chemist, a subject of the German Emperor, residing at 41 Rheinstrasse, Steglitz, near Berlin, Germany, have invented new and useful Improvements in Processes for the Manufacture of Color-Screens, of which the following is a specification.

My invention relates to the manufacture of color screens such as are used in three color photography. Screens of this kind consist of a transparent film, for instance a converted cellulose film the surface of which is divided into small portions stained according to the three fundamental colors. In manufacturing color screens of this kind it has been suggested to protect the surface of the film with a coating of a resinous or fatty substance such as for instance caoutchouc and to scratch narrow parallel lines in this protective coating by which the converted cellulose surface is exposed. If then the film is immersed in a bath containing a suitable staining solution, only those portions of the surface are stained which are exposed by the previous removal of the protective coating. In order to obtain the subsequent coloring it is necessary again to remove a part of the remaining protective coating. This can be done by again scratching out a system of parallel lines inclined at a suitable angle to the first system. The result then is a surface containing lines stained with the first color alternating with lines consisting of alternate fields covered with protective substance and fields having as yet no coloring. If this film is immersed in a staining bath some provision must be made to prevent the dye changing the coloring produced by the first bath. Then by washing in a suitable solvent the remainder of the protective coating can be removed and the film immersed for a third time in a staining bath.

I have discovered that a film stained by one dye, for instance a blue dye, is not affected by immersion in another dye for instance a green dye, if the solvent of the latter is made more dilute by the addition of water or other suitable liquids than that of the first dyeing solution. Accordingly my invention consists in providing a converted cellulose film with a protective coating which is successively changed to expose different portions of the surface and in suc-

cessively immersing the film in differently colored staining baths the solvents of which are progressively diluted for successive immersions.

The process can be carried out, for instance, in the following manner: A nitro-cellulose film is covered on both sides with a protective layer by dipping it into a solution of rubber in benzol, and in one of these layers a series of lines are scratched just deep enough to expose the cellulose surface. The film is then dipped into a solution of a blue dye stuff which is for instance obtained by dissolving 2 grams of Victoria blue in 100 cubic centimeters of absolute alcohol. The film is rinsed in water in order to wash off the excess of the dye. The protective layer is then again cut up into parallel lines preferably arranged at an angle of 90° to the direction of the first ruling, and these second lines also reach only to the surface. The nitro-cellulose surface will be thus decomposed into blue and noncolored lines, the latter of which are alternately decomposed into protected and unprotected squares. By dipping into a solution of 2 grams of auramin and 1 gram ethyl green in 150 cubic centimeters of alcohol of 80%, the unprotected parts will be colored green, while the portions already colored blue will remain unaffected owing to the greater dilution of the solvent. The remaining portions of the protective layer are then washed off from the film which now represents a screen consisting of blue lines and green squares and the third coloring can be effected with red dye stuff in a still more diluted solvent. To that end is used for instance a solution of 2 grams of rubin and 1 gram auramin in 150 cubic centimeters of alcohol of 60%. When the screen is treated with this stain only the non-colored portions will be stained. The result will therefore be a color screen consisting of blue lines and green and red squares, and the non-treated protective layer is then removed from the back of the said color screen in any well known manner.

The above example may be considered as typical inasmuch as it represents a very simple rule of proceeding. I find however that it is not equally applicable to different kinds of converted cellulose. Converted cellulose as used for photographic films differs largely. Broadly two classes can be dis-

cerned namely nitrated cellulose and acetylated cellulose. The former is usually mixed with camphor but the percentage of camphor used largely varies with different manufacturers.

5 I have found that the substances and concentrations mentioned above by way of an example give indifferent results unless a converted cellulose is used consisting of 10 nitrated cellulose with a high percentage of camphor. For converted cellulose poor in camphor I find that the pure alcoholic solutions diluted with water can be greatly improved by adding acetone besides water.

15 As a rule I find that the percentage of acetone in the solvent should be increased as the amount of camphor present in the converted cellulose diminishes. With acetylated cellulose which contains no camphor 20 the ratio of the amounts of alcohol to those of acetone can be diminished to zero, or what comes to the same, material of this kind can be treated with dyeing solutions in pure acetone diluted with water.

25 As an example of dyeing solutions applicable to nitrated cellulose which is poor in camphor I give the following:

*Blue dye.*—2 grams of Victoria blue are dissolved in 100 cubic centimeters of alcohol 30 of 95% and to 100 cubic centimeters of this solution are added 4 cubic centimeters of acetone and 4 cubic centimeters of water.

*Green dye.*—2 grams of ethyl green and 2 grams of auramin are each dissolved in 100 cubic centimeters of alcohol of 95%. 35 30 cubic centimeters of the first and 70 cubic centimeters of the second solution are mixed and to the mixture are added 8 cubic centimeters of acetone and 8 cubic centimeters of water.

40 *Red dye.*—2 grams of rubin and 2 grams of auramin are each dissolved in 100 cubic centimeters of alcohol of 95%. 50 cubic centimeters of the first and 50 cubic centimeters of the second solution are mixed and to the mixture are added 10 cubic centimeters of acetone and 12 cubic centimeters of water.

45 As an example of dyeing solutions applicable to acetylated cellulose I give the following:

50 *Blue.*—2 grams Victoria blue, 50 cubic centimeters acetone, 50 cubic centimeters water.

55 *Green.*—2 grams ethyl green, 45 cubic centimeters acetone, 55 cubic centimeters water.

60 *Red.*—2 grams rubin, 40 cubic centimeters acetone, 50 cubic centimeters water.

The invention is not limited to the above examples. For instance, instead of the protective layer of rubber, any other suitable protective layer could be selected for the purpose. Other solvents or other suitable dye stuffs can also be used. Finally the sequence of coloring may be modified. In the 65 same way any combination of three funda-

mental colors can be selected which is suitable for reproducing natural colors in color photography.

If color screens of this kind are to be manufactured in larger quantities it is not 70 convenient to produce the unprotected parts of the surface to be stained by first covering it with a protective coating and then removing parts of the coating by scraping or scratching out lines. It is preferable instead to print lines or any other suitable patterns on the film by means of a cylinder suitably engraved, as is well known in the art. In this case the process must be slightly modified. For instance a system of straight 75 parallel lines of some fatty or resinous substance adapted to protect the surface covered thereby against alcoholic and other solutions of dyes may first be printed on the surface. Then the parallel lines remaining 80 unprotected may be stained by immersion in a blue dye. Then the protective lines may be washed off in benzol or any other suitable solvent. The product of this first series of operations is a screen having alternate blue 85 and unstained parallel lines. On this may be printed a second system of protective lines crossing the blue lines at any suitable angle and the film may then be immersed in a green dye prepared according to my in- 90 vention as described above, so as to stain the uncolored parts of the exposed lines but not to affect the parts already stained blue. The second system of protective lines is then again washed off and the result of this sec- 95 ond operation is a film covered with blue lines and green squares alternately. This is finally immersed in a third dye solution prepared as described above and after washing and drying the screen will then be ready for 100 use. It will be understood that it is within my invention to apply two of the colors, say green and blue, in the manner described, 105 a third color having been applied previously, or being applied subsequently, as may be 110 desired.

Having now particularly described and ascertained the nature of my said invention and in what manner the same is to be performed, I declare that what I claim is:— 115

1. The improvement in the process for manufacturing color screens for color-photography on converted cellulose films by means of a protective coating which is pro- 120 gressively changed to expose different parts of the surface to the effect of staining solu- 125 tions which improvement consists in suc- cessively immersing the film in the different staining solutions, the solvents of which are progressively diluted.

2. The improvement in the process for manufacturing converted cellulose color screen films by means of a protective coating which is changed to expose different 130 parts of the surface for successive staining

operations which improvement consists in successively immersing the film in the different staining solutions the solvents of which contain progressively increasing percentages 5 of water.

3. The improvement in the process for manufacturing nitro-cellulose color screen films by means of a protective coating that is changed to expose different parts of the 10 surface for successive staining operations which improvement consists in successively immersing the film in alcoholic staining solutions of different colors using progressively increasing percentages of acetone and water 15 for successive coloring baths, the ratio of the quantities of acetone to those of alcohol being increased as the percentage of camphor contained in the nitro-cellulose is diminished.

4. A process for manufacturing nitro- 20 cellulose color screen films which process consists in partially covering the film with a protective coating immersing in a blue staining solution, the solvent of which is a mixture of alcohol, acetone and water, changing 25 the protective coating so as to expose different parts of the surface and immersing in a green staining solution the solvent of which contains a larger percentage of acetone and water than the preceding, removing 30 the remainder of the protective coating and immersing in a red staining solution the solvent of which contains a still larger percentage of acetone and water than the first mentioned one, the ratio of the percentage of 35 alcohol to that of acetone being decreased according to the percentage of camphor contained in the film.

5. A process for manufacturing nitro-cellulose color screen films which process consists in printing parallel lines of a protective 40 resist on the surface of the film, immersing in a solution of a blue staining substance in alcohol, acetone and water, removing the protective printing by washing in a solvent,

printing a second system of parallel lines of 45 protective substance inclined toward the first system on the surface of the film, immersing the film in a solution of a green staining substance in alcohol, acetone and water 50 employed being greater than with the blue solution, removing the protective printing by washing in a solvent and finally immersing in a solution of a red staining substance in alcohol, acetone and water, the percentage of 55 acetone and water in the solvent being greater than that used with the green staining solution, the percentage of acetone employed in the solvents being increased as the percentage of camphor contained in the film 60 diminishes.

6. A process for manufacturing three color screens on films of converted cellulose which process consists in printing on the 65 surface of the film parallel lines of a protective substance, immersing the film in a solution of a blue coloring substance in acetone and water, removing the protective printing by washing in a solvent, printing a second system of lines of a protective substance inclined to the first system, immersing in a solution of a green staining substance in acetone and water the percentage of water 70 being larger than with the blue solution, removing the protective printing by washing in a solvent and finally immersing the film in a solution of a red staining substance in acetone and water the percentage of water 75 being greater than that of the green staining solution.

In testimony whereof I have signed my name to this specification in the presence of two subscribing witnesses.

CARL SPÄTH.

Witnesses:

WOLDEMÄR HAUPT,  
HENRY HASPER.